

March 23, 1948.

W. M. CUTLER

2,438,150

SOAKING, FREEZING, AND DRYING BY SUBLIMATION OF UNTANNED HIDES

Filed April 22, 1944



Inventor

Wallace M. Cutler

By His Attorney

*Wallace M. Cutler*

## UNITED STATES PATENT OFFICE

2,438,150

SOAKING, FREEZING, AND DRYING BY  
SUBLIMATION OF UNTANNED HIDESWallace M. Cutler, Gloucester, Mass., assignor to  
United Shoe Machinery Corporation, Flemington, N. J., a corporation of New Jersey

Application April 22, 1944, Serial No. 532,270

5 Claims. (Cl. 8—94.15)

1

This invention relates to methods of treating untanned hides and skins and to the products produced thereby. More specifically the invention relates to methods of treating hides and skins which involve the steps of soaking and freezing an untanned hide or skin freshly removed from the carcass of an animal and then drying it at subfreezing temperatures to prepare it for subsequent operations, depending upon the nature of the product desired. Invention is also to be recognized as residing in both tanned hides or skins as well as in untanned hides or skins prepared as articles of commerce in accordance with the new method. It is to be understood that the method, when carried out, is not limited to the use of any particular machines and/or apparatus.

This application is a continuation in part of application Serial No. 367,055, filed November 25, 1940, which has matured into Patent No. 2,354,200 and is entitled "Method of drying hides and skins." In the present application, when "hides" alone are spoken of, both hides and skins are referred to, the purpose in using the single term being to eliminate verbiage.

It is an object of this invention to treat untanned hides in such a way that the untanned product will be improved as to ease and expense in handling, will be less subject to bacterial action with its consequent loss of hide substance and quality, and be more easily susceptible to subsequent tanning. Another object is to provide a method of hide treatment in which is eliminated the necessity of shipping or storing of untanned hides in salt and by such elimination to avoid shipping and storage charges on excess weight due to salt and water. A further object is to provide a method and product, both of which permit clean and pleasant working conditions for the personnel handling the hides. Still another object is to promptly stop putrefaction of fresh hides and, as a consequence, to avoid localized hide stains and general hide quality deterioration as well as actual loss in hide substance and area. Another object is to secure a light weight, high quality, untanned hide which can be packed, shipped, or stored or which, if it is desired, may be used for the manufacture of leather as soon as produced, the time of production being low. Still another object is to produce a preserved untanned hide which with a considerable saving in time may be subsequently tanned in a conventional manner or in the manner taught in the said Patent No. 2,354,200, referred to above. Another object is to combine the present improved method for producing an untanned hide with

2

any conventional tanning method or with the method disclosed in the said patent to secure an improved leather. Yet another object is the production of a tanned hide of excellent and improved quality with all its useful substance intact.

In the practice of my invention, a fresh untanned hide is first given a wash to remove foreign matter adhering to it in the slaughter house. In case excess flesh should remain on the hide, because of imperfections in the carrying out of the process of flaying, the hide is scraped to remove such flesh. Residual flesh will materially slow down the drying process if not removed. The hide is then soaked in water preferably containing some agent such as salt to aid in removing water-soluble proteins although that is not essential (such proteins do not form leather substance when a hide is subsequently tanned) and the soaked hide is then rinsed with water to cleanse the hide of such agent and/or other foreign matter. The hide then contains an appreciable amount of water and while in that condition is frozen. As a result of the freezing operation, the hide substance is expanded, due to the presence of ice crystals formed in the spaces or interstices between the fibers and fibrils of the hide substance. The rate of freezing is controlled in accordance with the characteristics of the product desired. Apparently the slower the freezing operation, the larger the ice crystals will be and hence the greater the expansion of the interstices or spaces in the hide substance, with the result that the slowly frozen hide results usually in being the plumper and softer hide as compared with a hide which is subjected to quick freezing. However that may be, the frozen hide is then dried by contacting it with a water-absorbing medium, the hide being maintained under subfreezing conditions with no or slight thawing being permitted. The drying should be largely by sublimation if the advantages of the present invention are to be achieved. Whereas a fresh or green hide or skin has a specific gravity of about 1.050 to about 1.075, the same hide dried by the method herein described has a much lower specific gravity and a calfskin correspondingly dried has a specific gravity of about .344 as will be seen in a table of test results to be subsequently referred to. Green hides and skins (containing, as is usual, more than one-half their weight in water after the flaying operation) which have been dried in the open air are hard or horny and much shrunken with a specific gravity of about .775 to about 1.40. Plump, light weight, soft and untanned hides produced by the

present method may be conveniently packaged or merely stacked and are preserved, because of their dryness, against bacterial action until subsequent treatment such as tanning is given them. Whether the tanning process be a conventional one or of the type disclosed by Patent No. 2,354,200, advantages such as a considerable saving in time and hide substance are secured in the carrying out of that process by using the untanned hides produced with the new method 10 herein disclosed.

These and other important advantages and characteristics of the method and of the products will now be described in detail in the specification and then pointed out more particularly in the appended claims.

In the drawing, the single figure is a diagrammatic flow sheet representing by way of example the steps of the new method and the order in which they may be followed.

Following the flow diagram the hide (promptly after removal from the animal carcass) is first given a preliminary wash and, if the flaying operation has been imperfectly carried out, the side is then "fleshed" or scraped to remove any excess flesh. It is then soaked in a water bath until its weight has appreciably increased and following that step, the hide is washed or rinsed to remove foreign matter. The water bath may have in it some agent such as common salt or sodium polysulphide to aid in removing water-soluble proteins from the untanned hides although use of such an agent is not essential. The washing or rinsing should remove any such agent to a substantial degree before the process is proceeded with. After being drained for a brief period, the hide is then promptly subjected to a freezing temperature condition to check any tendency toward putrefaction and to preserve such hide in its fresh condition. Preliminary to the freezing operation, the hide may be spread out on a smooth plate or it may be stretched on a frame although neither step is essential. The hair, which is a valuable product, is retained on the hide during the steps A through F on the diagram and has no deleterious effect in so far as the process is concerned. Having been frozen, the hides may be passed directly after freezing to a drying chamber wherein a water-absorbing medium, such as air, is brought in contact with the hide, the latter being retained under sub-freezing temperature conditions until it is dried to the desired degree such as to an "air-dry" condition, by sublimation of its water content. In order to insure that the moisture is removed from the hide by a process of sublimation, the temperature of the hide is conveniently kept at about 26° F. However, this temperature may be varied within a preferable range between about 30° F. and about -20° F. It is clear that drying performed at a temperature relatively high in the given range is more economical than at a lower temperature. This drying by sublimation may be carried out with the temperature of the flowing air or other drying medium being maintained even above that of the hide. The essential factor is that the drying is by sublimation and not by evaporation. It will be readily understood that the rate at which hides or skins are dried may be regulated by the amount, and the temperature, of air or gas circulated in the drying chamber, by the rapidity of its circulation, and by the amount of the air dehumidifying agent if such an agent is used. It will be understood also that the drying of a hide by this

method will not usually be continued to the point where it may be said to be "bone-dry," this for the reason that all hides and skins readily take up moisture from the atmosphere and vary in their water content from day to day. Hence, ordinarily, a hide will be dried to a point whereat it contains moisture in the range of about 8% to 13%, that is, until it reaches what may be termed an "air-dry" condition. A greater amount of moisture may be left in the hide but that amount should in no case be sufficient to promote bacterial growth or action.

As indicated above, a marked advantage of the present method of treating untanned hides 15 resides in the fact that such hides are preserved by the treatment, it being possible to store them and ship them under ordinary atmospheric conditions of temperature and humidity, care being taken (of course) to see that no water touches them. Hides placed in a dry or an "air-dry" condition will be preserved for an extensive period as the presence of at least 20% moisture is ordinarily essential for bacterial action. When it is recalled that, according to commonly practiced methods, hides and skins must be treated with large amounts of salt to preserve them for shipment to the tanners and that such hides and skins must be handled in bundles or in casks for which a special freight car must be employed, 20 because of the malodorous condition that prevails in spite of the most careful preservative treatment, it will be understood that very considerable expense has heretofore been involved in preserving hides and skins and in shipping them to the tanners. Furthermore, the tanner has had to provide a cool basement as a storage space for such hides or skins. Moreover, it often has been the practice, upon opening bundles of such hides or skins, to trim therefrom deteriorated and/or 25 damaged edge portions preliminary to the soaking operation which soaking operation is performed to remove the salt or other chemical and to bring back the hide or skin to a uniformly soft and clean condition. This soaking operation consumes from one to five days of time, with several changes of water, and constant supervision to avoid putrefactive changes due to bacterial action, which takes place rapidly with any rise in temperature of the water. In spite 30 of the care exercised by those responsible for the salting and/or other preservative treatment of green hides or skins and for the soaking operations, there is always a considerable loss of substance due to putrefactive changes and to hydrolysis of hide substance in the soaking operation.

It is a marked advantage of the drying method and the product disclosed herein that hides and skins thus dried are not only preserved against 35 putrefactive changes but because of their cleanliness and light weight they may be handled at a minimum of expense and, if desired, they may be conveniently packaged or stacked to facilitate the handling.

Another marked and important advantage of the method is that the time involved in carrying out steps A to F (see the flow sheet) in order to produce a hide ready for the tannery need not exceed 36 hours. Contrast this short period with the minimum period of 30 to 60 days which is essential to cure a hide for the tannery when it is packed in salt in the conventional manner used in this country.

The plump, untanned, freeze-dried hide or skin 40 has another advantage and that is appreciated

when the hide or skin is to be "wet back," which constitutes a preliminary essential step at the tannery. As it is plump and open in structure, it "wets back" quickly. It takes four or five days for an ordinary dry hide to "wet back" sufficiently for tanning. In the case of wet salted calfskins it takes from 10 to 12 hours. With wet salted hides it takes 20 to 25 hours. The following table of test-results shows that the first seven samples (which were produced by using applicant's process) are capable of rapid "wetting back" and are superior, in this respect, to wet salted hides. The last four columns of the said table of test-results serve to illustrate that the soaked and freeze-dried samples 1 to 7 were far superior to the horny samples 8 to 16 (not properly freeze-dried) in their ability to assimilate water:

for each method. In each method of tanning, however, it is essential that the untanned hide first be "wet back" or soaked and it is in this connection that the plump, freeze-dried and untanned hide facilitates the operations carried on in a tannery. In so far as the vegetable tanning is concerned, the drawing shows, by way of examples, the steps which may be taken in the treatment of hides to produce heavy or sole leather. Excellent chrome-tanned leather has been produced from a plump, freeze-dried calfskin by using a conventional method similar to that shown at the far left of the flow diagram. In the event that the method of tanning disclosed in the Patent No. 2,354,200 is used, soaking time is also saved and the entire process from the fresh hide to finished leather will involve two separate stages of drying by sublimation to yield excellent

| Sample | Wgt. Received, Grams | Soaking and Rinsing Time, Hrs. | Wgt. with Water | Drying Treatment | Wt. (Grams) Dried to 13% H <sub>2</sub> O Content | Density of Shaved Sample (13% H <sub>2</sub> O) | Appearance and Feel of Product | Per cent Pick-up in Weight of Shaved Sample Having 13% H <sub>2</sub> O Before Pick-up |     |     |      |
|--------|----------------------|--------------------------------|-----------------|------------------|---------------------------------------------------|-------------------------------------------------|--------------------------------|----------------------------------------------------------------------------------------|-----|-----|------|
|        |                      |                                |                 |                  |                                                   |                                                 |                                | Hours in Water at 72° F.                                                               |     |     |      |
|        |                      |                                |                 |                  |                                                   |                                                 |                                | 0.017                                                                                  | 1.0 | 2.0 | 24.0 |
| 1.     | 189                  | 72                             | 305             | Freeze Dried     | 94                                                | 0.3                                             | Firm White Plump               | 72.0                                                                                   | 211 | 215 | 225  |
| 2.     | 248                  | 91                             | 344             | do               | 101                                               | 0.3                                             | do                             | 150.0                                                                                  | 228 | 228 | 216  |
| 3.     | 246                  | 24                             | 358             | do               | 100                                               | 0.33                                            | do                             | 57.0                                                                                   | 202 | 212 | 216  |
| 4.     | 143                  | 62                             | 230             | do               | 58.5                                              | 0.255                                           | do                             | 178.0                                                                                  | 248 | 270 | 228  |
| 5.     | 220                  | 2.5                            | 285             | do               | 102.0                                             | 0.427                                           | do                             | 37.0                                                                                   | 148 | 167 | 177  |
| 6.     | 270                  | 19.0                           | 312             | do               | 102.0                                             | 0.45                                            | Firm Gray Plump                | 34.0                                                                                   | 170 | 208 | 190  |
| 7.     | 258                  | 66.0                           | 324             | do               | 104.0                                             | 0.345                                           | Firm White Plump               | 123.0                                                                                  | 212 | 212 | 236  |
| 8.     | 179                  | 0                              | 177             | do               | 110                                               | 0.805                                           | Horny                          | 7.0                                                                                    | 63  | 77  | 125  |
| 9.     | 173                  | 0                              | 173             | Air Dried        | 101                                               | 0.89                                            | do                             | 6.3                                                                                    | 63  | 81  | 125  |
| 10.    | 124                  | 0                              | 124             | do               | 61.5                                              | 0.85                                            | do                             | 5.7                                                                                    | 80  | 98  | 145  |
| 11.    | 141                  | 0                              | 141             | do               | 61                                                | 0.825                                           | do                             | 6.2                                                                                    | 74  | 103 | 153  |
| 12.    | 231                  | 0                              | 231             | do               | 109                                               | 0.90                                            | do                             | 4.9                                                                                    | 49  | 75  | 124  |
| 13.    | 204                  | 0                              | 208             | Freeze Dried     | 104                                               | 0.92                                            | do                             | 4.0                                                                                    | 47  | 61  | 114  |
| 14.    | 184                  | 0                              | 184             | Air Dried        | 89                                                | 0.72                                            | do                             | 6.2                                                                                    | 66  | 79  | 112  |
| 15.    | 223                  | 20.75                          | 303             | Freeze Dried ?   | 106                                               | 0.88                                            | do                             | 4.1                                                                                    | 44  | 71  | 118  |
| 16.    | 246                  | 48                             | 318             | do               | 103                                               | 0.92                                            | do                             | 3.6                                                                                    | 62  | 91  | 116  |

In analyzing the above table, it can be seen that samples 1 to 7 inclusive illustrate the fact that soaking and freeze-drying produce excellent results. It should be noted that samples 1 to 7 inclusive, when dried by applicant's method, had a density substantially below 0.72—that is, substantially below the lightest product made from samples 8 to 16 inclusive. Samples 8 and 13 show that freeze-drying without soaking is of no avail (other than, of course, that it inhibits bacterial action during the time the hide is frozen). Samples 9 to 12 inclusive and 14 illustrate that merely air-drying a hide will result in a horny product difficult to "wet back" for tanning purposes. Samples 15 and 16 show that results are not satisfactory if care is not taken that the hides are actually freeze-dried or dried by sublimation. In the latter samples, the agent (salt) was apparently not adequately washed out, with the result that the ice in the samples melted during the drying step. When this occurs, the open spacial structure of the hide is not maintained, yielding a horny product which will not readily receive moisture—i. e.—"wet back" rapidly.

When the plump untanned product has reached a tannery it may be treated in a number of ways, as shown by the flow sheet. It may be tanned by either the chrome or the vegetable tanning method. Each of these methods may be conventional or they may be as taught in the above-referred-to earlier Patent No. 2,354,200 and shown as the "Cutler method" in the flow sheet. It is to be understood that infinite variations in all these methods can be used and that only one of the many possible orders of steps are shown in the diagram

leather which has not been weakened at any stage of production by bacterial action, excessive shrinkage or violent treatment. In this latter method, the hide to be chrome tanned is maintained in a damp or wet condition during the conventional pretanning and tanning steps and also during fat liquorizing and coloring before it is again frozen and dried. If the hide is to be vegetable tanned, then it is kept wet during the unhairing, bating and tanning steps and then frozen and dried by sublimation to secure an excellent product.

Having described my invention, what I claim as new and desire to secure by Letters Patent of the

United States is:

1. A method of treating a fresh untanned hide which comprises soaking the hide in water to appreciably increase its weight, freezing the hide, and contacting the frozen hide with a water-absorbing medium while said hide is maintained under subfreezing conditions to dry the hide by sublimation.

2. A method of treating a fresh untanned hide which comprises soaking the hide in water to appreciably increase its weight, freezing the hide at a controlled rate dependent upon the characteristics of the product desired, and contacting the frozen hide with flowing air while said hide is maintained under subfreezing conditions to remove water from the hide by sublimation.

3. A method of treating a fresh untanned hide which comprises soaking the hide in water containing an agent to aid in removing water-soluble proteins, washing the hide with water to largely eliminate the agent, freezing the hide, and con-

tacting the hide with a water-absorbing medium while said hide is maintained under subfreezing conditions to dry the hide by sublimation.

4. A method of treating a fresh untanned hide to produce leather which comprises soaking the hide in water to appreciably increase its weight, freezing the hide, contacting the frozen hide with a water-absorbing medium under subfreezing temperature conditions to bring the hide to a condition sufficiently dry to inhibit bacterial action, and subsequently subjecting the dried hide to a tanning procedure.

5. An untanned substantially air-dry hide having a density substantially below 0.72, said hide being prepared in accordance with the method of claim 1.

5

10

15

WALLACE M. CUTLER.

### REFERENCES CITED

The following references are of record in the file of this patent:

#### UNITED STATES PATENTS

| Number    | Name   | Date          |
|-----------|--------|---------------|
| 2,102,699 | Green  | Dec. 21, 1937 |
| 2,354,200 | Cutler | July 25, 1944 |

#### FOREIGN PATENTS

| Number | Country       | Date |
|--------|---------------|------|
| 12,642 | Great Britain | 1905 |